

## UNITED STATES PATENT OFFICE

ELTON R. DARLING, OF DECATUR, ILLINOIS, ASSIGNOR, BY MESNE ASSIGNMENTS, TO CORNSTALK PRODUCTS COMPANY, INC., OF NEW YORK, N. Y., A CORPORATION OF DELAWARE

## METHOD FOR THE PRODUCTION OF PULP

No Drawing.

Application filed June 22, 1928. Serial No. 287,651.

This invention relates to the production of pulp suitable for any of the many uses for which pulp of the usual type is adapted, and has especial reference to the production of 5 pulp from many of what have been considered the wastes of agriculture containing a low lignin content and relatively high amounts of pentosans.

Among the vegetable growths in this class 10 may be included cornstalks, bagasse, rice, and wheat straw, together with corn cobs, oat hulls, rice hulls, cottonseed hulls, etc., etc.

There have been many methods devised for the pulping of these low lignin content and 15 high pentosan content materials; but as will be seen in the disclosure hereinafter, the method of this application is new, and involves great economy and features which permit of the production of specialty pulps and paper 20 at a great saving of time, labor and expense.

As is well known, the basic structure of the materials referred to hereinbefore is cellulose associated with other materials which can be separated from the cellulose in various ways, 25 some of which involve deterioration of the cellulose, and others of which involve drastic treatment. The latter treatment frequently deteriorates the cellulose as well as the structure thereof from a physical standpoint.

30 In the process of this application the treatment accorded the material is not drastic, the final product is obtained in a very satisfactory condition for many uses, and the cost of production is low, thereby permitting competition with other pulps produced at a low 35 cost, but lacking many of the desirable properties possessed by the cellulose obtained by this process.

In working some of the materials referred 40 to above, such as cornstalks, bagasse, etc., it is necessary to shred them to make them workable, and it has been found practical and desirable to co-ordinate a washing process with the said shredding process, so that dirt and 45 foreign matter collected in the field may be removed at the same time.

The shredded and washed material is then fed into a digester, ten times its weight in water is added, the digester is closed and heat 50 and pressure of approximately ten pounds is

applied. The digester used is constructed so that the water therein may be drawn out at the lower portion thereof, passed through a heater, and then sprayed into the top of the digester where it is sucked through the mass and again passed out of the digester at the bottom thereof. 55

This process is followed for a period of approximately thirty minutes, in which time any water soluble materials present are extracted and the fibre is opened and made more 60 susceptible to the subsequent treatments.

As is well known the plant growths referred to herein as used in this process contain two types of pentosans, one of which 65 types acts as reserve food material for the plant, the other type going to make up the structure of the plant, one of its functions being the binding together of the fibres. When these binding pentosans are treated 70 in a manner to convert them into soluble chemical products, their removal is not only easy, but frees the fibres, which may then be readily acted upon by certain chemicals to make the pulping operation easy of accomplishment. 75

This process of treating the pentosans may be termed hydrolysis and it has been found efficient and economical in the use of same 80 in connection with this process to employ a weak solution of sulphuric acid, for instance, one percent.

When the aforesaid hydrolysis operation is completed and pressure has been used, the pressure is released, the acid solution is 85 drained off, and the residual mass is washed to remove the acid.

The material is then in a condition to continue with the process disclosed in the co-pending patent application of Jackson and 90 Darling, Serial No. 280,646 filed May 25th, 1928.

I do not desire to limit myself strictly to the use of pressure in either the water soluble material extraction step, nor the hydrolysis step of this method, as satisfactory results 95 may be obtained without employing pressure, but the time of treatment is reduced, and under some conditions better results are attained when pressure is used. 100

Neither do I desire to be limited strictly to the use of sulphuric acid in the step of rendering soluble and removing the binding pentosans without damage to the fibre.

5 Other chemicals of a more costly nature could be used to equal advantage, but at greater expense, and, therefore, the sulphuric acid is preferable.

Having thus described my invention, what 10 I claim and desire to secure by Letters Patent, is:—

1. The method of producing cellulosic pulp from vegetable growths of low lignin content and relatively higher pentosan content 15 comprising the following steps; shredding and cleansing the material; digesting same in approximately ten times its weight of water and under heat and pressure; drawing off the water, heating same and passing 20 it through the material again; treating the material with a weak sulphuric acid solution; and removing the acid from the mass.

2. The method of producing cellulosic pulp from vegetable growths of low lignin content and relatively higher pentosan content 25 comprising the following steps; shredding and cleansing the material; digesting same in water, under heat, and under a pressure of approximately ten pounds; drawing off 30 the water, heating same and passing it through the material again; treating the material with a weak sulphuric acid solution; and removing the acid from the mass.

3. The method of producing cellulosic 35 pulp from vegetable growths of low lignin content and relatively higher pentosan content comprising the following steps; shredding and cleansing the material; digesting same in approximately ten times its weight 40 of water and under heat; drawing off the water, heating same and passing it through the material again; treating the material with a weak sulphuric acid solution; and removing the acid from the mass.

45 4. The process of preparing cellulosic pulp from vegetable growths of low lignin and relatively high pentosan content which comprises shredding and comminuting the same, removing water-soluble constituents 50 therefrom by digestion with hot water, and then hydrolyzing the pentosans therein contained.

5. In the treatment of cellulosic raw materials of the nature of cereal straws such 55 as cornstalks and the like, the steps of removing from said materials the water-soluble constituents thereof by means of pressure-digestion with hot water, and then solubilizing the pentosans therein contained.

60 6. The process as defined in claim 4, wherein in the hydrolysis is carried out by treatment with a weak acid solution comprising sulphuric acid.

65 7. The process as defined in claim 4, wherein in the hydrolysis is effected by means of an

acid solution containing substantially 1% of sulphuric acid.

8. The process of producing cellulosic pulp from cornstalks which comprises shredding and comminuting said cornstalks, treating the same under heat and pressure with water, treating said water-treated cornstalks with a 1% solution of sulphuric acid, removing said sulphuric acid, and thereupon treating the cornstalks with water to remove the materials solubilized by the said treatment with the sulphuric acid.

In testimony whereof I have hereunto affixed my signature.

ELTON R. DARLING.

80

85

90

95

100

105

110

115

120

125

130